

# UNITED STATES PATENT OFFICE

ALBERT PATTON, OF MCKEESPORT, PENNSYLVANIA.

## PROCESS OF REFINING METALS.

1,091,588.

Specification of Letters Patent. Patented Mar. 31, 1914.

No Drawing.

Application filed September 24, 1907. Serial No. 394,338.

To all whom it may concern:

Be it known that I, ALBERT PATTON, a citizen of the United States of America, residing at McKeesport, in the county of Allegheny and State of Pennsylvania, have invented certain new and useful Improvements in Processes of Refining Metals, of which the following is a specification.

My invention relates to the manufacture of steel and relates more particularly to a process of refining metals by means of which phosphorus, oxids, silicates, and other impurities are removed during the refining operation. In eliminating these elements or impurities in the manner herein set forth, I am able to produce a non-corrosive steel, containing as low as one-tenth of 1% manganese; I also produce a more ductile and easily welded metal; also a metal having the qualifications conducive to the manufacture of rails and products requiring high tensile strength.

To put my process into practice, I use the iron that has been blown in an ordinary Bessemeyer converter or the iron from an acid open hearth furnace, the carbon having been reduced to a low percentage (in the neighborhood of 4/100 of 1%) and the silicon and manganese reduced as low as possible.

The process consists of a number of steps which may vary to meet various conditions, but which, in general, are of similar character, these general steps being as follows: Pour into an acid lined intermediate receptacle, then pour from this receptacle into a basic-lined receptacle, care being taken not to allow the acid slag to enter the basic-lined receptacle, and adding to the basic-lined receptacle, before, and possibly when pouring, materials for making a basic slag.

Manganese is added when the desired character of the product requires. The effect of this relative arrangement of steps on the iron is substantially as follows: The pouring of the metal into the acid-lined intermediate receptacle has substantially the same effect as the well-known methods of refining, my process differing from these methods mainly in the subsequent treatment.

When pouring from the acid-lined intermediate receptacle, especial care is taken to retain the acid slag in this intermediate receptacle, thus reducing the amount of lime ( $\text{CaO}$ ) required to make a basic slag. The materials for making a basic slag, such as lime-stone ( $\text{CaCO}_3$ ),

fluorspar ( $\text{CaF}_2$ ), etc., are charged into the basic-lined receptacle before (and possibly when pouring) the metal is poured, and if oxids of iron is required, it will be mixed in with the basic materials, the amount required being determined by the amount of oxids in the bath, and the phosphorus to be removed; it is to be understood that where the metal has been blown or reduced to the point or near the point above referred to (with the carbon reduced to a low percentage and the silicon and manganese reduced as low as possible), the phosphorus in the bath is there as phosphoric acid ( $\text{P}_2\text{O}_5$ ), due to the phosphorus having more affinity for the oxygen than the carbon, silicon or manganese (as these have been so reduced) or the iron itself. When the metal is brought into contact with these basic materials, a basic slag is made at which time, oxids and other impurities are removed and the phosphorus, in the form of phosphoric acid ( $\text{P}_2\text{O}_5$ ) is absorbed by this slag. The heat is then ready to be poured directly into molds or into another receptacle for the convenience of handling the heat to the place of casting. The manganese or re-carburizer desired can be added in the basic-lined receptacle or in the receptacle to which the metal is poured from the basic-lined receptacle.

In this process, by introducing a portion of the material for making basic slag into the metal being poured into the basic receptacle, the slag is formed quickly and all of the lime is used, practically eliminating the presence of small particles of the unused materials in the slag.

The use of the oxids in the bath acts to reduce the phosphorus and make the slag, and if additional oxids are needed, I use only enough to reduce the phosphorus as desired, the carbon, manganese and silicon having been reduced to the desired amount in the vessel or acid furnace.

This process provides for a rapid refining operation.

I claim:

1. The method of manufacturing steel which consists in subjecting the product of a Bessemeyer converter or an acid open hearth furnace to a refining operation which includes the following steps: pouring the molten metal into an acid lined intermediate receptacle, then pouring from said receptacle into a basic-lined receptacle and retain-

ing the acid slag in the acid-lined receptacle, and adding basic materials in the basic-lined receptacle.

2. The method of manufacturing steel which consists in subjecting the product of a Bessemer converter or an acid open hearth furnace to a refining operation which includes the following steps: pouring the molten metal into an acid-lined intermediate receptacle, then pouring from said receptacle into a basic-lined receptacle and retaining the acid slag in the acid-lined receptacle, and adding materials for making a basic slag, said materials absorbing the oxids and impurities in the bath to make the slag.
3. The method of manufacturing steel which consists in subjecting the product of a Bessemer converter or an acid open hearth furnace to a refining operation which includes the following steps: pouring the molten metal into an acid-lined intermediate receptacle, then pouring from said receptacle into a basic-lined receptacle and retaining the acid slag in the acid-lined receptacle, adding basic materials in the basic-lined receptacle, and adding manganese to the molten metal.
4. The method of manufacturing steel which consists in subjecting the product of

a Bessemer converter or an acid open hearth furnace to a refining operation which includes the following steps: pouring the molten metal into an acid lined intermediate receptacle, then pouring from said receptacle into a basic-lined receptacle and retaining the acid slag in the acid-lined receptacle, adding basic materials in the basic-lined receptacle, and adding manganese to the bath in the basic-lined receptacle.

5. The method of manufacturing steel which consists in subjecting the product of a Bessemer converter or an acid open hearth furnace to a refining operation which includes the following steps: pouring the molten metal into an acid lined intermediate receptacle, then pouring from said receptacle into a basic-lined receptacle and retaining the acid slag in the acid-lined receptacle, adding basic materials in the basic lined receptacle, and adding the rebarburizer in the basic-lined receptacle.

In testimony whereof I affix my signature in the presence of two witnesses.

ALBERT PATTON.

Witnesses:

H. C. EVERETT,  
A. J. TRIGG.